

Patented Apr. 11, 1944

2,346,562

# UNITED STATES PATENT OFFICE

2,346,562

## METHOD OF REMOVING CARBONIZED OIL RESIDUE FROM MAGNESIUM ARTICLES

Herbert K. De Long, Midland, Mich., assignor to The Dow Chemical Company, Midland, Mich., a corporation of Michigan

No Drawing. Application November 7, 1940,  
Serial No. 364,691

2 Claims. (CL. 141—1)

This invention relates to a method of cleaning articles of magnesium and magnesium-base alloys.

In certain processes for fabricating articles from magnesium and magnesium-base alloys, as by rolling, extrusion, drawing, and the like, practice occasionally demands that lubricants, usually mineral or vegetable oils, be used to facilitate operation. These oils tend to coat the surface of the resulting articles. Then, if the article is heat-treated or otherwise subjected to elevated temperatures during or after the particular fabrication process involved, the oils are, in part, decomposed or oxidized by the combined action of heat, air, and the magnesium surface, and are converted to gummy, carbonized materials, which, for present purposes, may be termed "oil residues." These residues, which also may be formed when oil-coated magnesium articles are exposed to the atmosphere for long periods of time, tend to detract from the appearance and usefulness of the final product, and should be removed. However, wire brushing is virtually without effect on the oil residues, and ordinary alkaline cleaners and degreasing solvents, although they loosen the residues somewhat, do not remove them satisfactorily.

It is therefore an object of the present invention to provide a simple, inexpensive, and effective method of removing oil residues from articles of magnesium and magnesium-base alloys.

According to the invention, oil residues are removed from magnesium and magnesium-base alloy articles by subjecting the articles to the action of an aqueous alkaline solution of a tartrate. In so far as is known, any water-soluble salt of tartaric acid may be used in the process, alkali metal tartrates such as sodium tartrate, sodium bitartrate, and Rochelle salt having been found particularly suitable. The tartrate should preferably be present in the solution in a concentration between about 1 and about 5 per cent by weight, although other proportions are operable in most instances.

The tartrate solution may be made alkaline by any soluble basic-acting agent, although in general the stronger bases, such as trisodium phosphate, sodium carbonate, tetramethyl ammonium hydroxide, and the like, and especially the alkali

metal hydroxides, e. g. sodium hydroxide, are greatly to be preferred. The alkaline agent is ordinarily, though not necessarily, added to the solution in a proportion between about 1 and about 5 per cent by weight.

While the treating solutions ordinarily contain only the tartrate and the alkali as effective ingredients, other substances may be added without departing from the invention. Thus, in 10 cleaning articles having on their surface a considerable film of oil in addition to oil residues, it is desirable to add to the tartrate solution 0.5 to 2.0 per cent by weight or more of a soluble detergent, such as a soap or a salt of a sulfated higher aliphatic alcohol or of a sulfonated aromatic hydrocarbon.

In cleaning oil-residue coated magnesium and magnesium-base alloy articles, it is necessary only to dip the article in the cleaning solution for a 20 short time, and then to withdraw it and rinse it in water. When the solution is hot, as at 90°-100° C., a simple dip for 15 seconds to 2 minutes suffices to remove all the oil residue. However, if the solution is at room temperature, strong agitation and a longer dipping time are necessary for effective cleaning. If desired, instead of simply dipping the article in the solution it may be cleaned electrolytically, as by being made the cathode of a cell in which the alkaline tartrate 25 solution is the electrolyte.

It is to be understood that the foregoing description is illustrative rather than strictly limitative, and that the invention is co-extensive in scope with the following claims.

What is claimed is:

1. The method of removing carbonized oil residue from the surface of magnesium and magnesium-base alloy articles, which comprises subjecting the article to the action of an aqueous solution consisting essentially of water and between about 1 and about 5 per cent by weight of an alkali metal tartrate and between about 1 and about 5 per cent of an alkali metal hydroxide, thereafter rinsing and drying the article.
- 40 2. The method according to claim 1 wherein the alkaline tartrate solution is maintained at a temperature of 90° to 100° C.

HERBERT K. DE LONG.